

Dec. 27, 1955

C. J. TOBIN

2,728,657

PROCESS OF MAKING ZINC BASE ALLOYS

Filed Sept. 25, 1950

2 Sheets-Sheet 1



0.45% Si 0.45% Si 0.45% Si 0.45% Si 0.45% Si 0.45% Si  
0.00% Mn 0.10% Mn 0.30% Mn 0.45% Mn 0.70% Mn 0.90% Mn  
CAST } CAST } CAST } CAST } CAST } CAST }  
775°F } 775°F } 775°F } 775°F } 775°F } 775°F }

Fig. 1



0.60% Si 0.60% Si 0.60% Si 0.60% Si 0.60% Si 0.60% Si  
0.00% Mn 0.10% Mn 0.30% Mn 0.60% Mn 0.90% Mn  
CAST } CAST } CAST } CAST } CAST } CAST }  
775°F } 775°F } 775°F } 775°F } 775°F } 775°F }

Fig. 2



0.60% Si  
0.00% Mn  
CAST }  
825°F }

0.60% Si  
0.10% Mn  
CAST }  
825°F }

0.60% Si  
0.30% Mn  
CAST }  
825°F }

0.60% Si  
0.60% Mn  
CAST }  
825°F }

0.60% Si  
0.90% Mn  
CAST }  
825°F }

Fig. 3



0.45% Si  
0.45% Mn  
CAST }  
825°F }

0.45% Si  
0.70% Mn  
CAST }  
825°F }

Fig. 4

Inventor

Clarence J. Tobin

Willits, Helwig & Baillio

Attorneys

Dec. 27, 1955

C. J. TOBIN

2,728,657

PROCESS OF MAKING ZINC BASE ALLOYS

Filed Sept. 25, 1950

2 Sheets-Sheet 2



Fig. 5



Fig. 6

Inventor

Clarence J. Tobin

By  
Willits, Blumig & Trallie

Attorneys

1

2,728,657

## PROCESS OF MAKING ZINC BASE ALLOYS

Clarence J. Tobin, Detroit, Mich., assignor to General Motors Corporation, Detroit, Mich., a corporation of Delaware

Application September 25, 1950, Serial No. 186,534

2 Claims. (Cl. 75—178)

The present invention relates to an improved alloy for drawing dies and to a process for producing such an alloy.

In the forming of metal shapes from sheet metal where the final form of the part requires a substantial amount of metal deformation, as, for example, in the forming of the various contoured parts of the body assembly of automotive vehicles, it is common practice to use drawing dies of cast iron or steel. Such dies are especially resistant to wear and while expensive, are used extensively in the automotive industry where large quantities of a shaped part are formed. Where, however, the part may not be required in large numbers, the initial expense of cast iron or steel drawing dies is prohibitive. Accordingly, there has been considerable demand for a material having suitable characteristics for drawing dies and less expensive in initial costs. An alloy which has found extensive use in the aircraft industry as a drawing die alloy for forming shaped parts from aluminum is the zinc base alloy containing copper, aluminum and magnesium and commonly known as "Kirksite". Where such dies have been used to make shaped metal parts from metals other than aluminum they have not been entirely satisfactory.

Accordingly, it is an object of the present invention to provide an improved zinc base alloy for drawing dies.

It is another object of the present invention to provide a low cost zinc base drawing die alloy.

It is still another object to provide a process for making such a zinc base alloy.

The alloy and the process for making the same which I desire to protect herein are specified with particularity in the appended claims and are described in the following specification. The drawings comprise Figures 1, 2, 3 and 4 illustrating macrographic views of the alloy of the present invention and Figures 5 and 6 illustrate in a cross-sectional view and a perspective view a typical drawing die made from such an alloy.

In accordance with one aspect of the present invention an exceptional combination of strength and wear resistance is obtained in zinc base alloys for drawing dies by controlled additions of silicon or silicon with manganese.

I have found that the controlled addition of silicon or silicon with manganese to a zinc base alloy containing aluminum, copper, magnesium with the balance zinc provides a dispersion of hard particles within the alloy which makes it particularly wear-resistant and especially suitable for use in drawing dies. In this connection it is believed that the desirable wear-resistance properties result from the formation of hard particles of silicon or an inter-metallic compound of manganese and silicon.

The addition of silicon alone to a zinc base alloy of the above composition will produce hard particles in the matrix which improves its wear-resisting properties to a considerable degree. In this connection it is believed that these particles are substantially pure silicon containing not more than a minor percentage of other metals in solution as impurities. As metallic silicon can be added

2

to the zinc rich alloy only with considerable difficulty because of the low solubility of silicon in solid and liquid zinc, it is preferably added as a hardening alloy of aluminum-silicon. The molten zinc will dissolve the aluminum from the hardening alloy and reject the silicon, leaving the silicon in the molten zinc as solid hard particles. Because these particles of solid substantially pure silicon present in the zinc rich base alloy have a substantially lower specific gravity than the zinc rich molten alloy 10 they tend to float to the surface of the molten alloy and a heterogeneous material results.

With the addition of manganese to the zinc base alloy containing silicon, the manganese combines with the silicon to form hard particles of substantially higher specific 15 gravity than the pure silicon particles, and consequently the tendency for floating and separation of the hard particles is lessened. Further, manganese when present with silicon in the zinc base alloy has no detrimental effect on the wear-resistance of the alloy. Its desirable function appears to be in obtaining a more suitable distribution 20 of the hard particles in the molten alloy prior to solidification. I have found that it is preferable to add the manganese to the zinc in the form of a copper-manganese alloy hardener.

25 The silicon may also be added to the zinc rich molten alloy as a copper-silicon alloy hardener. However, in adding the silicon in this manner the dissociation of the copper from the silicon by solution of the copper in the zinc is not complete and the remaining copper-silicon particles do not provide the wear-resisting characteristics obtained by the addition of silicon alone or in the form of the aluminum-silicon alloy hardener.

30 The zinc base alloys which I have found to have an exceptional combination of strength and wear-resistance in drawing dies contain substantially .2 to 1.2% silicon, 2.0 to 4.5% aluminum, .5 to 4.0% copper, .05 to .25% magnesium with the balance substantially all zinc. As pointed out heretofore, a more desirable dispersion of the hard particles is obtained when the above alloy contains substantially .1 to 1.2% manganese. The alloys which I have found preferable for drawing die alloys contain .45 to .75% silicon, .45 to .90% manganese, 2.0 to 4.5% aluminum, .5 to 4.0% copper, .05 to 25% magnesium with the balance substantially all zinc. Optimum characteristics of castability, strength and wear-resistance are obtained with alloys containing .45% silicon, .70% manganese, 2.75 to 3.50% copper, 3.75 to 4.25% aluminum and .05 to .25% magnesium.

35 The forming of the drawing die alloy of the present invention may be accomplished in different manners. However, I have found that improved characteristics are obtained where as a first step commercially pure zinc or mixtures of commercially pure zinc and scrap alloy of the "Kirksite" type are mixed together and melted in a separate furnace. The temperature of the molten material is brought to a temperature of 825 to 875 degrees Fahrenheit while at the same time a copper-manganese alloy hardener is melted in a separate furnace and brought to a temperature of substantially 1750 to 2000 degrees Fahrenheit. The molten alloy hardener is then added to the molten zinc or zinc and "Kirksite" mixture. At this stage I have found it desirable to remove any dross that is formed at the surface of the melt. This is accomplished by the addition of a flux such, for example, as ammonium 40 chloride. The addition of the ammonium chloride reduces the metal oxides and leaves a resultant ash or dross which is skimmed from the surface. With the melting of the zinc or zinc and scrap "Kirksite" alloy and the copper-manganese alloy hardener a second hardening alloy of aluminum-silicon is melted in still another furnace and brought to a temperature of 1300 to 1500 degrees Fahrenheit. The second alloy hardener is subsequently added to 45

the molten mixture of zinc or zinc and scrap Kirksite alloy and the copper manganese hardening alloy. Finally, magnesium in the form of rods, bars or ingots is added by submerging it below the surface of the bath and allowing it to dissolve. Constant agitation of the molten mixture is desirable during all of the alloying operations and in the ladle before casting.

Where the melting of the alloy is initiated with commercially pure zinc and additions of scrap alloy of the Kirksite type it will be appreciated that the chemical compositions of the alloy hardeners will be adjusted to obtain the desired composition in the final product. In this connection it might be added that when scrap metal is used the best results are obtained by limiting the scrap metal to 50% by weight of the initial melt of scrap metal and commercially pure zinc.

The alloy is cast into drawing die shapes preferably in green sand open molds through gates which enter the mold near the bottom. Heat is applied to the exposed liquid metal surface so that the metal will solidify from the bottom of the casting upwardly. To compensate for shrinkage, molten metal is added to the top of the casting as shrinkage occurs during solidification. To avoid or reduce segregation of the hard particles during casting it has been found desirable to heat the molten metal to a temperature of substantially 775 to 825 degrees Fahrenheit with a casting temperature of substantially 10 to 15 degrees above the melting point of the alloy being preferred. Under these conditions of casting the molten metal will be sufficiently viscous upon entering the mold to provide for a substantially even distribution of the hard particles throughout the casting. However, in the casting of large shapes the temperature should be raised as the lower casting temperature does not permit sufficiently free flow of the molten liquid to prevent uneven shrinkage and warping in the casting.

In the drawings the macrographic views of Figures 4, 5 and 6 illustrate the dispersion of the hard particles of silicon or the intermetallic compound of silicon and manganese in the zinc rich matrix.

Alloys such as I have described have unusual characteristics of strength and wear-resistance which make them particularly useful and desirable for drawing die alloys in drawing die operations where the initial expense of cast iron or steel drawing dies is prohibitive.

What I claim and desire to secure by Letters Patent of the United States is:

1. The process of making a drawing die of a zinc base

alloy characterized by a high degree of wear-resistance and consisting essentially of .5 to 4.0% copper, 2.0 to 4.5% aluminum, .2 to 1.2% silicon, 1.0 to 1.2% manganese, .05 to .25% magnesium with the balance zinc which comprises as the first step heating zinc to a temperature of substantially 825 to 875 degrees F., adding thereto a copper-manganese alloy which has been heated to substantially 1750 to 2000 degrees F., adding thereto an aluminum-silicon alloy which has been heated to substantially 1300 to 1500 degrees F. and thereafter adding magnesium and casting said zinc base alloy at a temperature of substantially 10 to 15 degrees F. above its melting temperature.

2. The process of making a drawing die of a highly wear-resistant zinc base alloy characterized by a dispersion therein of hard particles of an intermetallic compound of manganese and silicon and consisting essentially of approximately 2% to 4.5% aluminum, 0.5% to 4% copper, 0.05% to 0.25% magnesium, 0.2% to 1.2% silicon, 0.1% to 1.2% manganese and the balance zinc plus incidental impurities, said process comprising the steps of melting zinc, aluminum and copper together and heating to a temperature of approximately 825 to 875 degrees F., adding thereto a molten copper-manganese alloy heated to a temperature of about 1750 to 2000 degrees F., subsequently adding a molten aluminum-silicon alloy heated to a temperature of 1300 to 1500 degrees F., thereafter adding magnesium, and finally casting the molten metal at a temperature of approximately 10 to 15 degrees F. above the melting temperature of the resultant zinc base alloy.

#### References Cited in the file of this patent

#### UNITED STATES PATENTS

|           |               |               |
|-----------|---------------|---------------|
| 1,596,761 | Peirce et al. | Aug. 17, 1926 |
| 1,815,479 | Morrell       | July 21, 1931 |

#### FOREIGN PATENTS

|         |               |               |
|---------|---------------|---------------|
| 411,557 | Great Britain | June 12, 1934 |
| 420,672 | Great Britain | Nov. 30, 1934 |
| 429,021 | Great Britain | May 21, 1935  |
| 351,744 | Italy         | Aug. 20, 1937 |
| 522,724 | Great Britain | June 25, 1940 |

#### OTHER REFERENCES

Iron Age, Aug. 3, 1944, pages 46-49; 132, 134.